

H. J. HAON,  
PROCESS FOR THE PRODUCTION OF ARTIFICIAL PATENT LEATHER AND PRODUCT THEREOF,  
APPLICATION FILED FEB. 9, 1915.

1,372,021.

Patented Mar. 22, 1921.



Inventor  
Harry J. Haon  
By his Attorney  
Prindle, Wright & Sharpe

# UNITED STATES PATENT OFFICE.

HARRY J. HAON, OF NEWBURGH, NEW YORK, ASSIGNOR, BY MESNE ASSIGNMENTS, TO  
E. I. DU PONT DE NEMOURS AND COMPANY, A CORPORATION OF DELAWARE.

## PROCESS FOR THE PRODUCTION OF ARTIFICIAL PATENT-LEATHER AND PRODUCT THEREOF.

1,372,021.

Specification of Letters Patent. Patented Mar. 22, 1921.

Application filed February 9, 1915. Serial No. 7,146.

To all whom it may concern:

Be it known that I, HARRY J. HAON, of Newburgh, in the county of Orange and in the State of New York, have invented a certain new and useful Improvement in Processes for the Production of Artificial Patent-Leather and Products Thereof, and do hereby declare that the following is a full, clear, and exact description thereof.

10 My invention relates to the production of an artificial patent leather upon backings other than leather, as for example, cloth backings.

Hitherto attempts to produce artificial 15 patent leather by applying coatings to cloth have been unsatisfactory and unsuccessful, owing to the fact that the weave of the cloth invariably showed through the surface of the coating, even when the coating was 20 rather heavy, so that in order to hide the weave of the cloth it became necessary to apply an abnormally large amount of the coating material. The product containing the large quantity of the coating material 25 was impractical not only because of the cost of the materials required, but because of the great weight of the product.

The object of my invention is to produce 30 an artificial patent leather upon a cloth backing in such a manner as to hide the weave of the cloth, without the above disadvantages. In general this is accomplished by applying a coating to a woven fabric, then embossing the coated fabric with a 35 suitable grain, and thereafter applying one or more additional coatings until the grain is partially or entirely obscured by the coatings.

My invention is capable of embodiment 40 in many different forms, but for the purpose of illustration I shall refer only to certain forms thereof herein.

In the drawings—

Figure 1 represents diagrammatically an 45 apparatus adapted to carry out my process, and

Fig. 2 shows an exaggerated cross sectional view of a fabric coated in accordance with my process.

50 I may make use of any of the coating materials ordinarily used, as for example, pyroxylin, solvents, oil and pigment, or oil in combination with pigment. In order to give a patent leather finish to the product

I may apply oil alone, such for example as 55 linseed oil, or the oil mixed with pyroxylin and a dye. Any suitable kind of woven fabric may be used in carrying out my invention.

As one example of carrying out my invention I may proceed as follows:

Duck or heavy sateen is fed from the unbatching roll 1 to doctor blade 2, by means of which a coating of a mixture comprising 60 castor oil, pyroxylin and pigment mixed in suitable proportions and dissolved in a solvent, such as acetone or amyl-acetate, is applied until the materials deposited (as represented at 10) amount to form three to six 65 ounces of solid per square yard. The surface of the coated material is now embossed in a suitable shallow grain, such as a pebble or skiver. Thereafter similar coatings 70 are applied by doctor blade 5 until a total of about nine to twelve ounces of solids for 75 each square yard have been applied, and until the grain has been almost or entirely obscured. A finish coating 12 is then applied to the coated fabric by doctor blade 7 so as to give a high gloss, such as that obtained on patent leather. This finishing 80 coat may contain any of the materials ordinarily applied in the production of artificial leather, that is to say, pyroxylin, linseed oil and dye dissolved in amyl-acetate. In applying the coating material the same may be 85 spread over the fabric by the use of a doctor-knife, a brush, a slicker, or in any other suitable way. A tough, elastic material is thus obtained, in which the clothly appearance 90 is obscured, while at the same time the weight of the coating is not excessive. The product, furthermore, resembles patent leather very closely. Numerals 3, 6 and 8 denote suitable solvent recovery apparatus. 95

While I have described my invention above in detail, I wish it to be understood that many changes may be made therein without departing from the spirit of my invention.

I claim:

1. The process which comprises applying a coating material to a woven fabric, embossing the coated fabric to obtain a grain sufficient to hide the appearance of clothiness, 105 and then applying to the same side of the fabric a further quantity of a permanent coating material.

2. The process which comprises applying a coating material to a woven fabric, embossing the coated fabric, and then applying to the same side of the fabric a further quantity of coating material until the grain is entirely obscured.
3. The process which comprises applying a coating material to a woven fabric, embossing the coated fabric to obtain a grain sufficient to hide the appearance of clothiness, and then applying to the embossed surface a further quantity of a permanent coating material, the final coating being a finishing material to give a high gloss.
- 10 4. The process which comprises applying a coating material to a woven fabric, embossing the coated fabric, and then applying a further quantity of coating material until the grain is entirely obscured, the final coating being a finishing material to give a high gloss.
- 15 5. An artificial patent leather comprising a cloth backing, an embossed coating thereon having a grain sufficient to hide the appearance of clothiness, and a further permanent coating located over the embossed coating.
- 20 6. An artificial patent leather comprising a cloth backing, an embossed coating thereon having a grain sufficient to hide the appearance of clothiness, and a further permanent coating located over the embossed coating, the outer coating being a finishing coat to give a high gloss.
- 25 7. An artificial patent leather comprising

a cloth backing, an embossed coating thereon, and a further coating located over the embossed coating and obscuring the embossed coating, the outer coating being a finishing coat to give a high gloss.

40

8. The process which comprises applying a coating material to a woven fabric, embossing the coated fabric to obtain a grain sufficient to hide the appearance of clothiness, and then applying to the embossed surface a further quantity of coating material until the grain is largely hidden.

9. The process which comprises applying a coating material to a woven fabric, embossing the coating fabric to obtain a grain sufficient to hide the appearance of clothiness, and then applying to the embossed surface a further quantity of a coating material until the grain is largely hidden, the final coating being a finishing material to give a high gloss.

10. The process which comprises applying to a cloth backing a coating of material insufficient to obscure the clothiness of the fabric, embossing the coated fabric to obtain a grain sufficient to hide the appearance of clothiness, and applying a finish coating over the embossed surface.

In testimony that I claim the foregoing I have hereunto set my hand.

HARRY J. HAON.

Witnesses:

HARRY A. PIPER,  
CHAS. E. McSHANE.